

July 29, 1930.

A. BERNSTEIN

1,771,390

TWISTING AND REELING ARTIFICIAL SILK

Filed July 13, 1929



Inventor:  
Arnold Bernstein  
By  
A. J. Hedlund  
His ATTORNEY

## UNITED STATES PATENT OFFICE

ARNOLD BERNSTEIN, OF MANNHEIM, GERMANY, ASSIGNOR TO ZELLSTOFFFABRIK WALDHOF, OF MANNHEIM-WALDHOF, GERMANY

## TWISTING AND REELING ARTIFICIAL SILK

Application filed July 13, 1929, Serial No. 377,956, and in Germany March 15, 1928.

The invention relates to the twisting and reeling of artificial silk or the like and more particularly to artificial silk which is already wound on twisting spools in a damp condition.

5 In the production of artificial silk in accordance with the reeling process the filaments expressed through fine openings out of a thick liquid substance such as viscose are led direct into a coagulating liquid. The 10 cellulose tissues which result are wound on rotating spools, bobbins, or similar devices and subsequently undergo a long washing process in order to remove the adhering acids 15 and salts. The washed spools are dried, the artificial silk filament is twisted off and finally reeled.

This process is inconvenient, tedious, and requires a large number of bobbins and further, on account of the diverse and separate operations which are necessary a large expenditure of operating power is necessary.

In certain cases the freshly spun unwashed viscose filament is twisted off direct from the bobbins and is guided on to reels, the filament 25 on its passage from the bobbins to the reels being passed through the washing liquid in order to remove the adherent impurities. During such a process the rotating bobbin is 30 continuously subjected to the action of water spray and the twisted filament is guided on to the reels by means of filament guides located in the atmosphere.

During the twisting process by virtue of 35 the centrifugal movement the damp filament drawn off the twisting bobbins loses a part of its moisture and becomes sticky so that on its passage through the filament guides certain parts of the filament more easily adhere 40 to the guides thus producing breakages of the filament and rendering the artificial silk of poor quality.

One object of the invention is to provide a 45 method of twisting and reeling spooled damp artificial silk which avoids the adherence of the individual filaments to one another.

A further object of the invention is to provide a method of twisting and reeling spooled 50 damp artificial silk wherein the silk is sub-

mitted to a washing and protective action prior to reeling.

The method of the present invention consists in drawing off the filament from a twisting spool, allowing the drawn off twisted filament to fall direct into a liquid without the interposition of a guide surface or the like, guiding the filament by a guide member immersed in the liquid and winding the filament thus guided on a reel.

As the filament guide is located beneath the level of liquid, adherence of the filament to the guiding surface cannot take place. In order to prevent the inconvenient crystallizing out of salts on the bobbins during the 65 rotation thereof it is preferred to use for the spinning process precipitants which, as far as possible, do not crystallize out.

As the artificial silk when damp is especially sensitive to mechanical treatment it is 70 preferred to add to the liquid through which the filament passes substances adapted to form protective layers on the filament during its passage therethrough such as wax-oil emulsions.

75 The invention is more particularly described with reference to the accompanying diagrammatic drawing.

Referring to the drawing *a* denotes the 80 twisting bobbin which is located at the lower end of a rotating shaft driven by means of a belt or the like. The filament is drawn off the bobbin *a* over the head thereof and is drawn down by means of the rotating reel *d* at the same time being correspondingly 85 twisted. The filament falls freely into a steeping bath *c*, passes through a filament guide or guides *b* in the liquid over the guide *b* and is wound up on the reel *d* in the form of a skein.

90 The damp artificial silk hank thus wound on the reel is unbound, removed from the reel, washed and prepared in the usual manner.

95 What I claim is:—

1. A method of treating a spooled damp artificial silk filament which comprises removing the damp filament from the spool while rotating the spool to impart twist to the filament, winding the filament on a reel,

guiding the filament between the reel and the spool by means of a guide immersed in a liquid body and providing unconstrained movement of the filament from the spool to the liquid body.

- 5 2. A method of treating a spooled damp artificial silk filament which comprises removing the damp filament from the spool while rotating the spool to impart twist to  
10 the filament and disengaging moisture from the filament due to centrifugal action, winding the filament on a reel, guiding the filament between the reel and the spool by guides including a first guide immersed in a body of  
15 liquid adapted to form a protective layer on said filament and providing unconstrained movement of the filament from the spool to the liquid body.

In testimony whereof I have affixed my  
20 signature.

ARNOLD BERNSTEIN.

25

30

35

40

45

50

55

60

65